

## UNITED STATES PATENT OFFICE

HILTON IRA JONES, OF WILMETTE, ILLINOIS

## PROCESS AND MEANS FOR TREATING FABRICS

No Drawing.

Application filed March 14, 1927. Serial No. 175,441.

My invention relates to improvements in process and means for treating fabrics for rendering them waterproof, moth-proof, mildew-proof, mold-proof, and insect repellent.

An object of my invention is to provide a process for treating fabrics which does not involve the use of inflammable materials, thereby providing a treatment which can be carried out without any fire hazard.

10 A further object is to provide an economical process in which the only solvent employed is water.

A further object is to provide a process which will result in a product entirely free from the stickiness and greasiness which is so characteristic in the ordinary waterproofing treatments where oils, waxes, metallic soaps and the like are employed in hydrocarbon oil solvents.

15 A further object is to provide a means for treating textiles so as to increase their wearing qualities and at the same time making them hold their shape better as in the case of folded or pleated goods.

20 Other objects and advantages will appear in the following specification, and the novel features of the invention will be particularly pointed out in the appended claims.

25 In carrying out my invention, I provide two solutions, which I will term "A" and "B", respectively. As an example of the solution "A", I may use the following:

30 15 parts of soap  
10 parts of casein (put into solution with borax)  
5 parts carrageen (from Irish moss)  
30 parts bentonite  
500 parts petrolatum  
40 2400 parts water.

The soap, casein, carrageen which in this process act as auxiliary emulsifying agents and water are beaten together, a small amount of borax having been added to render the casein soluble. The temperature of the water should be preferably from 140° to 200° F. This forms an emulsion and into this smooth emulsion the bentonite is slowly sifted with continued stirring. When this

has been perfectly incorporated, the melted petrolatum is slowly added, the liquid being continuously beaten.

More or less water may be used within wide limits. It will be understood that this is given only as an example. Many different colloidalizing agents may be used in varying proportions, the essential ingredient being the colloidalized clay or bentonite. Without this, such permanent emulsions can be secured by such emulsifying or colloidalizing agents only in case they are relatively very concentrated—more in the nature of salves than solutions. Sodium alginate may be also used as a colloidalizing agent, while beeswax, carnauba wax, paraffin, lanolin and the like can be put into a permanent colloidal emulsion which will not separate on long standing, even though quite dilute. Any of these latter could therefore be used in lieu of the petrolatum without departing from the spirit of the invention. Furthermore, other materials, such as ochres, dry pigments and dyes, as well as fireproofing materials such as sodium silicate and sodium tungstate, may be incorporated without destroying the character of the colloidal emulsion. Also, very much larger proportions of oils and waxes may be used, if desired.

35 As an example of solution "B", I may give the following:

|                      |          |
|----------------------|----------|
| Cerium chloride----- | 1 part   |
| Water-----           | 40 parts |

This, as it will be observed, is a solution of a metallic salt. The salts of such metals as lead, copper, mercury, bismuth, thallium, and the like, or of other rare-earth metals, such as thorium, lanthanum, and of the radioactive metals, especially uranium, may be used.

45 The fabric, such as canvas, to be treated is immersed and thoroughly wetted with the "A" solution, then wrung out and passed at once into the "B" solution, then washed in water to remove excess metallic salts, wrung and dried.

50 In the example given above where petrolatum is used, it will be noted that as much as three-fourths of the entire weight of the

solids deposited upon the cloth is petrolatum, and yet the finished goods is wholly without any greasiness. This, as may be understood, is a highly desirable property. One result is that the goods remain cleaner than where the greasiness or stickiness tends to catch and retain dirt. All the ingredients as well as the finished product are odorless.

By suitable modification, such as using white waxes and colloidalizing agents, it is possible to leave the appearance of the treated goods entirely unchanged, but at the same time to render them water, moth, mildew and mold-proof, and in case salts of the radioactive metals are used, highly repellent to cockroaches, ants, bed-bugs and the like. As stated above, the treatment actually makes the goods wear longer, since the nap is less easily rubbed off and the goods hold their shape and press better. Another feature is that goods so treated are light instead of being dark and gloomy as is the case of tents treated in the ordinary ways to render them waterproof.

In lieu of the natural colloidalized clay or bentonite, I may use artificially colloidalized clay, made by grinding the clay with a dilute solution of tannic acid.

I claim:-

1. The herein described steps in a process of treating textiles, which consist in forming an emulsion containing petrolatum kept in suspension by the conjoint action of bentonite and an auxiliary emulsifying agent, wetting the textile with the emulsion, and subsequently treating the textile with a solution of a rare earth chloride, whereby a salt of the rare earth chloride is precipitated in the textile.

2. The herein described steps in a process of treating textiles, which consist in forming an emulsion containing petrolatum kept in suspension by the conjoint action of bentonite and an auxiliary emulsifying agent, wetting the textile with the emulsion, and subsequently treating the textile with a solution of a rare earth salt, whereby a salt of the rare earth metal is precipitated in the textile.

3. The herein described steps in a process of treating textiles, which consist in forming an emulsion containing petrolatum kept in suspension by the conjoint action of an equal proportion of bentonite and auxiliary emulsifying agents, wetting the textile with an emulsion, and subsequently treating the textile with a solution of a rare earth salt, whereby a salt of the rare earth is precipitated in the textile.

HILTON IRA JONES.